

Sept. 14, 1926.

**1,599,561**

**A. B. EMERY**

### CONCENTRATION OF ORES

Filed Dec. 5, 1922

2 Sheets-Sheet 1



Sept. 14, 1926.

1,599,561

A. B. EMERY

CONCENTRATION OF ORES

Filed Dec. 5, 1922

2 Sheets-Sheet 2



INVENTOR

Augustus B. Emery

BY

Jennie, Davis, Marvin, Edmonds

ATTORNEYS

## UNITED STATES PATENT OFFICE.

AUGUSTUS BACHELDER EMERY, OF MESSINA, TRANSVAAL, SOUTH AFRICA.

## CONCENTRATION OF ORES.

Application filed December 5, 1922, Serial No. 604,987, and in South Africa September 21, 1922.

This invention relates to the concentration of ores, and has for its object the provision of a new and improved method of and apparatus for the concentration of ores by flotation.

The present invention contemplates certain improvements in the present customary methods of concentrating ores by flotation. In general, these methods involve the fundamental feature of producing a froth possessing selective attraction or preference for the metalliferous particles of an ore pulp in contradistinction to the gangue particles thereof. For the formation of the froth, air or other appropriate gas is essential and in the present customary methods of flotation, such air is obtained by agitation or aeration or by a combination of aeration and agitation of the ore pulp. The improvements contemplated by the present invention involve more particularly an improved method of and improved apparatus for bringing about the necessary inter-action between the ore pulp and air or other appropriate gas for the production of a mineral-bearing froth.

In accordance with one aspect of the present invention, an ore pulp, containing an appropriate flotation agent, is caused, in the presence of air or other appropriate gas and in the form of a multiplicity of small separated streams or jets, to impinge against a baffling surface with sufficient violence to effectively break up the ore pulp streams and thereby form a mineral-bearing froth. Thus, the separated streams or jets of ore pulp may be projected against a baffling surface adapted to effectively break up or atomize the same in a gas-filled space, which may advantageously be a space containing atmospheric air. The mineral-bearing froth so formed is in accordance with the preferred practice of the invention trapped beneath the surface of the main body of the ore pulp and is recovered from a relatively quiescent zone of the main body of ore pulp. Preferably, the ore pulp is circulated within an appropriate receptacle in the course of which circulation the ore pulp is elevated to a height above the normal operating ore pulp level in the receptacle and discharged back into the receptacle in the form of relatively fine streams which are intercepted by the surface of the ore pulp in the receptacle or by

an appropriately positioned baffle with sufficient violence to effectively break up the ore pulp streams in the presence of air or other appropriate gas with the attendant formation of a mineral-bearing froth. 60

The improved apparatus of the invention is especially adapted for the practice of the method of the invention. This apparatus comprises an elongated vessel divided into a plurality of receptacles or cells in each of which is provided appropriate means for effecting a circulation of ore pulp in a path substantially at right angles to the direction of flow of the ore pulp through the vessel. The circulation of 70 the ore pulp in each receptacle or cell of the apparatus is carried out in the manner which characterizes my improved method of flotation, that is, with the elevation of the ore pulp, preferably pneumatically, to a height above the normal operating ore pulp level in the receptacle and the discharge of the so elevated ore pulp in the form of relatively fine streams against a baffling surface with sufficient violence to 80 form a mineral-bearing froth. 75

The foregoing and other novel features of the invention will be better understood from the following description taken in conjunction with the accompanying drawings, in which. 85

Fig. 1 is an elevation partly in section of the improved apparatus of the invention;

Fig. 2 is a sectional elevation of the apparatus of Fig. 1 taken on the section line 90 2-2;

Fig. 3 is an elevation partly in section of the discharge end of the apparatus;

Fig. 4 is a partial top plan of the apparatus; 95

Figs. 5 and 6 are detail views illustrating the construction of the pneumatic pulp-elevating means.

The improved apparatus illustrated in the accompanying drawings comprises an elongated vessel 10 divided longitudinally by transverse partitions 11 into a plurality of separate receptacles or cells. Thus, the vessel may be divided into ten (or more or less) such receptacles. The partitions 11 are constructed in two parts with an appropriate space 12 between the upper and lower parts to permit of the desired flow of ore pulp from one receptacle to the next. In cross section, the vessel 10 is V-shaped. 110

in its lower portion and rectangular in its upper portion.

An oblong shaped conduit formed by side members 13 and end members 14 is centrally disposed in each receptacle of the vessel 10. The lower end of each conduit is open and in free communication with the receptacle near the bottom thereof, while the upper end terminates in a box having a plurality of orifices or nozzle openings 15 in each side thereof and closed at the top by a cover 48. The oblong conduits are longitudinally disposed in their respective receptacles and are guided into their operative positions by guide cleats 45 secured to the partitions 11 and guide blocks 46 on the lower flared portions of the conduits. The conduits are suspended or hung in position by means of strips or bars 47 secured to the end members 14 of the conduit and resting upon the tops of the partitions 11. The side members 13 are outwardly flared at their bottoms so as to catch all of the air discharged from the air distributor as hereinafter more fully described.

A pipe 16 is centrally disposed in each of the oblong conduits and terminates at its lower end in a cylindrical air distributor 17. The pipes 16 are connected at their upper ends to an air supply main 25.

Each air distributor 17 is made up of a cylindrical tube 18 having its ends closed by circular caps 19 held together by a bolt 20. The tube 18 is provided with a plurality of holes 21. The perforated tube 18 is externally surrounded by one or more layers 22 of fine wire screen or loosely woven cloth such, for example, as burlap, or gunny-sack cloth. A clamping frame 23 serves to operatively connect the air distributor to the pipe 16 whereby the interior of the tube 18 is placed in communication with the pipe 16.

The air distributors 17 rest upon the bottoms of the receptacles in the vessel 10 and are held in their operative positions by means of guide blocks 24. The air distributors are positioned directly beneath the lower open and flared ends of their respective oblong conduits.

A vertical partition or baffle 26 is arranged on each side of the oblong conduit in each of the receptacles of the vessel 10. The partitions 26 are operatively held in place between a fixed cleat 27 and a removable cleat 28, the latter being held in position by the clamping action between a fixed tapered block 29 and a removable tapered block 30. The lower ends of the partitions 26 extend a short distance below the normal operating ore pulp level in their respective receptacles and serve to divide each receptacle (on each side of the central oblong conduit) into an inner froth-forming compartment and an outer froth-collecting compartment.

Each side of the vessel 10 is provided with

launders 31 for collecting and carrying away the froth overflowing the sides of the froth-collecting compartments of each receptacle. The froth overflow height of any froth-collecting compartment may be appropriately adjusted by means of removable strips 32 operatively held in position by the clamping action of a fixed tapered block 33 and a removable tapered block 34.

The launders 31 are preferably arranged to separately collect the froth overflow of particular receptacles. Thus, the froth overflow from certain receptacles near the feed end of the vessel may be separately collected from the froth overflow from the other receptacles of the vessel.

A pair of feed pipes 35 are arranged for the introduction of ore-pulp into the first receptacle at the feed end of the vessel. At the discharge end of the vessel, the ore pulp flows from the last receptacle into a compartment 36. The compartment 36 has an overflow discharge at its top, the height of which may be adjusted by means of removable strips 37. The bottom of the compartment 36 is provided with a discharge opening adapted to be closed by a valve 38. The overflow discharge from the compartment 36 flows into a box 39 which is suspended by means of a rod 40 and spring 41 and which has, at its lower end, a discharge spigot 42. A lever arm 43 is secured at one end to a fixed part of the vessel 10 and at its other end to the box 39 and intermediate its ends to the valve 38. A discharge pipe 44 is provided for carrying away the tailings discharged through the bottom opening in the compartment 36 and the spigot 42 in the suspended box 39.

In carrying out the improved method of the invention in the apparatus illustrated in the accompanying drawings, a suitably prepared ore pulp containing an appropriate flotation agent is introduced into the first receptacle or cell of the vessel 10 through the feed pipes 35. Air or other appropriate gas, under suitable pressure, is introduced into the air distributors 17 and enters the ore pulp in a relatively fine state of subdivision directly beneath the flared lower end of the oblong conduit in each receptacle. The air rising in these conduits exercises an air lift action and causes an upward flow of ore pulp through the conduits with the attendant discharge of the ore pulp through the nozzles or orifices 15. The ore pulp is discharged through the orifices or nozzles 15 in the form of a multiplicity of small separated streams or jets which impinge upon the surfaces of the partitions or baffles 26 or the top surface of the main body of ore pulp in the receptacles, or both, and are thereby effectively broken up or atomized in a gas-filled space with the formation of a substantial froth. The froth thus formed

- is at once driven downwardly and outwardly under the bottom edge of the partitions 26, and the froth then rises in the froth-collecting compartment on the other side of the partitions 26 and overflows into the launders 31. The remainder of the ore pulp from which the sulfides have been in large part eliminated (by being caught in the froth) circulates towards the bottom of the receptacle and in part passes on to the next succeeding receptacle and in part is again picked up by the air lift action in the oblong conduit and again ejected through the nozzles 15. It will thus be seen that the ore pulp gradually works its way through the successive receptacles of the vessel 10 passing through the openings 12 in the partitions 11 and being repeatedly circulated in each receptacle in the manner described.
- 10 The tails are discharged from the last receptacle into the compartment 36 where the sands settle out and drop through the automatically operated valve 38, while the slimes and water rise and overflow the adjustable 15 weir 37 into the movable box 39. If the ore pulp level in the vessel 10 rises the overflow into the box 39 will increase and this increased overflow will not be able to escape through the spigot 42 and the box will fill, 20 thereby increasing the weight of the box and contents. This increased weight will compress the spring 41 and will open more widely the valve 38, thus increasing the discharge of tailings through the bottom opening 25 in the compartment 36, and consequently lowering the pulp level in the vessel. If the pulp level in the vessel falls, the reverse action takes place. This automatic discharge device maintains the desired pulp level in the vessel 10 and has the advantage of not requiring any hand regulation or attention and of not blocking on account of an excess of sands.
- 30 After the froth has been formed in the froth-forming compartment of my improved apparatus by the action of the impinging jets of ore pulp, these same jets of ore pulp may break down the froth, unless it is at once removed out of their way. 35 This removal of the froth is accomplished in my improved apparatus by means of the arrangement of the partitions 26, which provide adjacent but separate froth-collecting compartments into which the froth is driven promptly after its formation. The lower edge of the partition 26 being beneath or substantially beneath the normally operating ore pulp level, serves to trap the froth so that it cannot return to the point where the jets of ore pulp impinge upon it. The froth is thus preserved as fast as formed, and because of its lightness, can be built up by increments of additional froth until it overflows the froth-collecting compartment 40 into the cooperating launder. No froth is entirely stable and the gas bubbles in the froth are constantly breaking down. At the same time new froth is constantly being formed. The new froth crowds in from below, thus forcing up the gas bubbles remaining unbroken and thus there occurs a continuous discharge of froth into the launder placed to receive it.
- 45 It is important to be able to accurately and conveniently control the rate of production and discharge of froth. If the production is too rapid, the froth will not "clean itself" and will carry over, with the concentrates, a considerable amount of waste or tailing material. The froth, when first made in the froth-forming compartment of my improved apparatus, is composed of bubbles which carry concentrates mixed with gangue. When these bubbles break the 50 adhering particles are dropped and the bubbles just below pick up by preference the sulfide particles, letting the gangue particles fall further down until they finally reach and mix with the ore pulp. By regulating the production and discharge of the 55 froth, the amount of "cleaning" can be controlled and preferential concentration by flotation can be promoted. In my improved apparatus, if a great volume of froth is produced, the velocity of the rising column of 60 froth is rapid and the time available for cleaning the froth by the break-down of part of the bubbles is reduced so that the bubbles can carry over not only various 65 sulfides but also gangue.
- 65 Even with a rapid production of froth, the cleanliness of the froth can be controlled by the rapidity of discharge. If the vertical froth column is extended so that a column of froth of great height is required before 70 a discharge over a lip at the top of the column can take place, then the bubbles will have to travel a long distance before discharged, and a greater opportunity will be afforded for the bubbles to break down and thus clean the froth. Furthermore, the great height of the column will increase the pressure of the bubbles, also tending to break 75 them down. But most important of all is the fact that the material dropped by the 80 upper bubbles has a deep column of bubbles to pass through before it reaches the pulp, hence more opportunity for the sulfides to be caught by bubbles before finally reaching 85 and becoming lost in the pulp.
- 85 While I prefer to effect the circulation of the ore pulp pneumatically by the air lift action hereinbefore described, any other equivalent means may be employed. For example, an ordinary hydraulic pump, 90 capable of handling acid or alkaline liquors, may be used if desired. The air-lift pump circulates the ore pulp rapidly with no wear and tear or moving mechanical parts; it 95 requires very little attention; and there is 100

very little abrasion from coarse sands when the latter are treated. Moreover, while I prefer to introduce the air into the ore pulp through a coarsely woven cloth, such as gunny-sack cloth, in order to finely disseminate the air, this is not necessary and the air may, if desired, be introduced into the ore pulp in larger masses for effecting the desired air lift action and the attendant circulation of the ore pulp.

The improved apparatus of the invention enables a number of treatments to be given in a single vessel with suitable provision for controlling simply and accurately the discharge of concentrates from each treatment operation independently of the other treatment operations.

The improved apparatus of the invention is well adapted for the practice of differential flotation. The discharge of concentrates from any one receptacle may be entirely stopped while continuous circulation of the ore pulp is maintained therein, thus enabling the mixing of freshly added flotation agent with the circulating ore pulp.

Owing to the absence of moving parts and owing to the fact that a sloping bottom is not depended upon for moving the sands in the pulp, the improved apparatus of the invention can be successfully used for concentrating 20 mesh or even coarser sands without causing trouble by the sands banking. Moreover, in my improved apparatus, a constant pulp level is maintained throughout in each of the receptacles without any regulating device for the individual receptacles, the ore pulp simply flowing without throttling or other regulation from one receptacle to the next.

From the foregoing description it will be evident that I have provided a flotation apparatus having a plurality of cells in each of which the ore pulp is separately circulated with the formation of a mineral-bearing froth. This mineral bearing froth is formed by streams or jets of ore pulp impinging against the surface of the ore pulp or against baffles or both. The froth so formed is driven into a froth-collecting compartment where it is trapped and prevented from returning into the froth-forming compartment. In the froth-collecting compartment, the froth accumulates and builds up, being caused to flow upwards (in a vertical column) before it is discharged with the object of "cleaning" the froth by the continual breaking of a part of the "bubbles" resulting in the material carried by the broken bubbles being successively reselected by falling on the unbroken bubbles below.

I claim:

1. The method of concentrating ores by flotation which comprises circulating an ore pulp within an appropriate receptacle and in the course of such circulation elevating

the ore pulp to a height above the normal pulp level in the receptacle, discharging the so elevated pulp back into the main body of pulp in the form of a multiplicity of small separated streams so that the streams of pulp impinge against a baffling surface with sufficient violence to atomize the streams of pulp in a gas filled space and form a mineral bearing froth, and recovering the mineral-bearing froth so formed. 75

2. The method of concentrating ores by flotation which comprises passing an ore pulp through an elongated receptacle divided into a plurality of chambers in each of which chambers there is maintained a circulation of ore pulp in a path substantially at right angles to the general direction of flow of ore pulp through the receptacle and in the course of which circulation the ore pulp is elevated to a height above the normal pulp level in the receptacle, discharging the so elevated pulp back into the main body of pulp in the form of a plurality of small separated streams so that the streams of pulp impinge against a baffling surface with sufficient violence to effectively break up the streams of pulp in a gas-filled space and form a mineral-bearing froth, and recovering the mineral-bearing froth so formed. 85 90

3. The method of concentrating ores by flotation which comprises circulating an ore pulp within an appropriate receptacle and in the course of such circulation elevating the ore pulp to a height above the normal pulp level in the receptacle, discharging the so elevated pulp back into the main body of pulp in the form of a plurality of small separated streams so that the streams of pulp impinge against a baffling surface with sufficient violence to effectively break up the streams of pulp in a gas filled space and form a mineral-bearing froth, promptly removing the mineral-bearing froth from the zone of its formation and preventing its return to such zone by trapping the froth within a relatively quiescent zone of ore pulp and permitting the froth to rise therein and form a froth column above the ore pulp in said quiescent zone, and recovering the mineral-bearing froth from said froth column. 100 110 115

4. The method of concentrating ores by flotation which comprises passing an ore pulp through an elongated receptacle divided into a plurality of chambers in each of which chambers there is maintained a circulation of ore pulp in a path substantially at right angles to the general direction of flow of ore pulp through the receptacle and in the course of which circulation the ore pulp is elevated to a height above the normal pulp level in the receptacle, discharging the so elevated pulp back into the main body of pulp in the form of a multi- 120 125 130

- plicity of small separated streams so that the streams of pulp impinge against a baffling surface with sufficient violence to atomize the streams of pulp in a gas-filled space and form a mineral-bearing froth, promptly removing the mineral-bearing froth from the zone of its formation and preventing its return to such zone by trapping the froth within a relatively quiescent zone of ore pulp and permitting the froth to rise therein and form a froth column above the ore pulp in said quiescent zone, and recovering the mineral-bearing froth from said froth column. 75
5. The method of concentrating ores by flotation which comprises pneumatically elevating from a body of ore pulp a column thereof, discharging the pulp near the top of the column in the form of a multiplicity of small separated streams against a baffle adapted to atomize the streams of pulp in a gas-filled space and thereby forming a mineral-bearing froth, and recovering the mineral-bearing froth so formed. 80
20. 6. The method of concentrating ores by flotation which comprises pneumatically elevating from a body of ore pulp a column thereof, discharging the ore pulp near the top of the column in the form of a multiplicity of small separated streams, causing said streams of ore pulp to impinge against a baffling surface with sufficient violence to atomize said streams in a gas-filled space and thereby forming a mineral-bearing froth, trapping the mineral-bearing froth so formed beneath the surface of the body of ore pulp, and recovering the mineral-bearing froth from a relatively quiescent zone of said body of ore pulp. 85
40. 7. The method of concentrating ores by flotation which comprises subjecting an ore pulp in the presence of an appropriate flotation agent to continuous retreatment by elevating from a body of the ore pulp a column thereof, continuously discharging the ore pulp near the top of said column in the form of a multiplicity of small separated streams, causing said streams of ore pulp to impinge against a baffling surface with sufficient violence to effectively break up said streams in a gas-filled space and thereby form a mineral-bearing froth, returning the mineral-bearing froth and associated ore pulp to said body of ore pulp and trapping the mineral-bearing froth beneath the surface thereof, and recovering the mineral-bearing froth from a relatively quiescent zone of said body of ore pulp. 90
45. 8. An apparatus for concentrating ores by flotation which comprises a receptacle adapted to contain ore pulp, means for circulating the ore pulp in said receptacle and for elevating the circulating ore pulp to a height above the normal operating pulp level within the receptacle, means for discharging the ore pulp so elevated back into the receptacle and against a baffling surface in the form of a multiplicity of small separated streams so that the streams of ore pulp are caused to impinge against said baffling surface with sufficient violence to atomize up the streams of pulp in a gas-filled space and thereby form a mineral-bearing froth, and froth-collecting means operatively associated with the receptacle. 95
50. 9. An apparatus for concentrating ores by flotation which comprises an elongated receptacle having a plurality of communicating chambers arranged to permit the flow of ore pulp from one end of the receptacle through said chambers to the other end of the receptacle, means associated with each of said chambers for circulating the ore pulp in the chamber in a path substantially at right angles to the general direction of flow of ore pulp through the receptacle and for elevating the circulating ore pulp to a height above the normal operating pulp level within the receptacle, means for discharging the ore pulp so elevated back into the receptacle and against a baffling surface in the form of a multiplicity of small separated streams so that the streams of ore pulp impinge against said baffling surface with sufficient violence to atomize the streams of pulp in a gas-filled space and thereby form a mineral-bearing froth, and froth-collecting means operatively associated with the receptacle. 100
55. 10. An apparatus for concentrating ores by flotation which comprises a receptacle adapted to contain ore pulp, means for elevating ore pulp from within the receptacle to a height above the normal operating ore pulp level within the receptacle, means for discharging the ore pulp so elevated back into the receptacle in the form of a multiplicity of small separated jets, means whereby in the operation of said apparatus such discharged jets of ore pulp are caused to impinge against a baffling surface with sufficient violence to break up the jets in a gas-filled space and form a mineral-bearing froth, and froth-collecting means operatively associated with the receptacle. 105
60. 11. An apparatus for concentrating ores by flotation which comprises a receptacle adapted to contain ore pulp, means for circulating the ore pulp in said receptacle in the course of which circulation the ore pulp is elevated to a height above the normal operating ore pulp level in the receptacle and discharged back into the receptacle in the form of a multiplicity of small separated jets, means cooperating with the aforementioned circulating means whereby in the operation of the apparatus said discharged jets of ore pulp are caused to impinge against a baffling surface with sufficient violence to break up the jets in a 110
65. 12. 125
70. 130

gas-filled space and form a mineral-bearing froth, and froth-collecting means operatively associated with the receptacle.

12. An apparatus for concentrating ores by flotation which comprises a receptacle adapted to contain ore pulp, an upright conduit within the receptacle having a lower open end near the bottom of the receptacle and terminating at its upper end in a plurality of relatively small orifices at a height above the normal operating ore pulp level within the receptacle, means for effecting an upward flow of ore pulp in said conduit, and froth-collecting means operatively associated with the receptacle.

13. An apparatus for concentrating ores by flotation which comprises a receptacle adapted to contain ore pulp and having a froth-forming compartment and a froth-collecting compartment communicating therewith below the normal operating ore pulp level in the receptacle, means for circulating the ore pulp in said receptacle in the course of which circulation the ore pulp is elevated to a height above the normal operating ore pulp level in the receptacle and discharged back into the receptacle in the form of a multiplicity of small separated jets, means whereby in the operation of said apparatus such discharged jets of ore pulp are caused to impinge against a baffling surface adapted to atomize the jets of ore pulp in a gas-filled space, and froth-collecting means operatively associated with said froth-collecting compartment.

14. An apparatus for concentrating ores by flotation which comprises a receptacle adapted to contain ore pulp, an upright conduit within the receptacle having a lower open end arranged near the bottom of the receptacle and terminating at its upper end in a plurality of relatively small orifices at a height above the normal operating ore pulp level within the receptacle, said orifices being adapted to direct ore pulp discharged from the upper end of said conduit back into the receptacle, pneumatic means operatively associated with said conduit for effecting an

upward flow of ore pulp therein, means whereby the ore pulp discharged through said orifices is caused to impinge against a baffling surface within the receptacle, and froth-collecting means operatively associated with the receptacle.

15. An apparatus for concentrating ores by flotation which comprises a receptacle adapted to contain ore pulp, an upright baffle arranged to provide in the upper part of the receptacle, a froth-collecting compartment and a froth-forming compartment communicating therewith below the normal operating ore pulp level in the receptacle, means for circulating the ore pulp in said receptacle in the course of which circulation the ore pulp is elevated to a height above the normal operating ore pulp level in the receptacle and discharged in the form of a multiplicity of small separated streams into the froth-forming compartment of the receptacle, means whereby in the operation of said apparatus such discharged streams of ore pulp are caused to impinge against said baffle, and froth-collecting means operatively associated with said froth-collecting compartment.

16. An apparatus for concentrating ores by flotation which comprises a receptacle adapted to contain ore pulp, an upright conduit within the receptacle having a lower open end near the bottom of the receptacle and terminating at its upper end in a plurality of relatively small orifices at a height above the normal operating ore pulp level within the receptacle, means for introducing into the lower open end of said conduit air in a state of relatively fine subdivision and thereby effecting an upward flow of ore pulp through the conduit and out of the orifices thereof, means whereby in the operation of said apparatus the ore pulp ejected from said orifices impinges against a baffling surface and thereby forms a mineral-bearing froth, and froth collecting means operatively associated with said receptacle.

In testimony whereof I affix my signature.  
AUGUSTUS BACHELDER EMERY.